

## UNITED STATES PATENT OFFICE

2,319,822

## COMPOSITION FOR IMPROVING THE ABSORBING PROPERTIES OF FABRICS AND THE LIKE

Warren L. Moody and Stanley J. Wagar,  
Richmond, Va.No Drawing. Application August 30, 1940,  
Serial No. 354,908

5 Claims. (Cl. 8—132.5)

This invention relates to wetting and penetrating agents and particularly to the processing of fabrics to impart to them the property of increased ability to wipe faster due to their greater affinity for water.

One of the objects of the invention is the treatment of fabrics and particularly new fabrics, such as towels, wiping rags and other water absorbing materials with certain specified inorganic salts whereby the fabrics are immediately usable as wiping agents. A towel treated as hereinafter set out has immediate wipability and it is not necessary to launder this towel or other treated fabric four or five times by commercial laundering processes to render the towel or other fabric suitable as a wiping medium.

A still further aim of the invention is the impregnation of a towel or other fabric with a finely adjusted balance of acid and alkaline inorganic salts whereby the treated fabric fibre has imparted thereto properties which decrease surface tension and lower contact angle of liquids coming in contact therewith and increase capillarity of the fibres themselves.

According to the instant invention materials may be impregnated during the course of their manufacture, or manufactured articles may be impregnated or the impregnation may be effected even when laundering used articles.

As illustrative of one manner of treatment, bottom bleached, piece bleached or gray goods is passed under a roll in an immersion box containing a solution formed of the following ingredients in the proportions indicated:

|                                                          | Parts    |
|----------------------------------------------------------|----------|
| Water (pH of which is 7) -----                           | 35 1,000 |
| Monosodium phosphate -----                               | 4        |
| Slaked lime (not less than 97% $\text{Ca(OH)}_2$ ) ----- | 1        |

The solution prepared as above will have a pH of not more than 6.8.

After treatment the fabric is carried to a dryer and the chemicals absorbed are fixed in the fabric. The above solution may be used in conjunction with wetting out agents such as soaps, alcohols, esters, sulphonated fatty alcohols, glycols or sulphonated products as the last operation and drying in the fabric as a finish to gain immediate wipability.

It will be understood that other alkaline or alkali earth phosphates may be employed in lieu of the monosodium phosphate and other alkali earth hydroxides may replace the slaked lime. However, it is of importance that the pH of the final solution does not exceed 6.8.

The above solution when applied to textile fabrics and other fibers impregnates itself into the material and is not dissipated by dry heat as are other materials. The advantages of the instant process may be set out as follows:

1. Treated fabrics are immediately wettable.

60

- 2. By drying faster the effects of any abrasion is reduced and increased life of the fabric results.
- 3. The use of the salts in solution as in a dye bath intensifies shades or colors.
- 5 4. Dyed goods will have their colors intensified when passed through a solution made according to the disclosed invention.
- 5. White goods are made whiter by this treatment.
- 10 6. Gray goods are improved in color and appearance by the disclosed composition.
- 7. Fabrics processed as disclosed have wiping qualities far surpassing those of untreated new goods.
- 15 8. No laundering or washing is necessary as fabrics, such as towels, have immediate usability.
- 9. No breaking in is necessary.
- 10. No objectionable feel on hand.
- 11. Impregnates, but does not load the goods.
- It is to be understood that while the invention is described specifically with regard to vegetable fibres and textile articles produced therefrom, it is applicable to other vegetable materials, and to porous inorganic materials generally, to animal fibers and synthetic yarns, that is to say, to any material having absorptive properties which it is desired to improve. It is contemplated to cover all such and to be limited in this respect only as may be necessary by the scope of the claims hereto appended.

What we claim and desire to secure by Letters Patent is:

1. A method of treating textile materials to improve their absorbent properties comprising impregnating said materials with a water solution of mono-alkali phosphate and an alkali earth hydroxide the pH of the solution being not more than 6.8.

2. A method of treating textile materials to improve their absorbent properties comprising impregnating said materials with a water solution of mono-alkali phosphate and slaked lime, the pH of the solution being not more than 6.8.

3. A method of treating textile materials to improve their absorbent properties comprising impregnating said materials with a water solution of monosodium phosphate and slaked lime, the pH of the solution being not more than 6.8.

4. A textile impregnating solution composed of water, monosodium phosphate and slaked lime, the pH of the solution being not more than 6.8.

5. A textile impregnating solution composed of the following ingredients in the approximate proportions indicated:

|                                                          | Parts |
|----------------------------------------------------------|-------|
| Water (pH of which is 7) -----                           | 1,000 |
| Monosodium phosphate -----                               | 4     |
| Slaked lime (not less than 97% $\text{Ca(OH)}_2$ ) ----- | 1     |

WARREN L. MOODY.  
STANLEY J. WAGAR.